

# UNITED STATES PATENT OFFICE.

ARTHUR SAMUEL O'NEIL, OF WILMINGTON, DELAWARE, ASSIGNOR TO E. I. DU PONT DE NEMOURS AND COMPANY, OF WILMINGTON, DELAWARE, A CORPORATION OF DELAWARE.

## PROPELLENT EXPLOSIVE.

1,311,910.

Specification of Letters Patent. Patented Aug. 5, 1919.

No Drawing.

Application filed August 17, 1916. Serial No. 115,452.

*To all whom it may concern:*

Be it known that I, ARTHUR SAMUEL O'NEIL, of Wilmington, in the county of New Castle, and in the State of Delaware, 5 have invented a certain new and useful Improvement in Propellant Explosive, and do hereby declare that the following is a full, clear, and exact description thereof.

My invention relates particularly to a 10 smokeless powder which has received a surface treatment so as to produce what is known as a progressive powder, that is to say, a powder which produces a lower initial pressure without lowering the velocity of 15 the projectile. My invention is applicable to the various kinds of rifle and cannon powders.

The object of my invention is to produce 20 a powder of this character which avoids many of the disadvantages of previous 25 powders of this type. More particularly, the object of my invention is to provide a powder of this character which is obtained by applying to the surface of powder grains, 30 as for example, grains of nitrocellulose powder, a deterrent material which is a solvent of the explosive contained in the powder grains so that it may be caused to penetrate the powder grains, and which is 35 substantially non-volatile and which, further, provides on the surface of the grains an explosive of sufficient potential to obtain satisfactory ignition. A further object of my invention is to provide a material for 40 application to the surface of the powder grains which has substantially no odor, and which is so slightly volatile that the powder produced in accordance with my invention may be stored at the temperatures to which 45 powders are ordinarily subjected without producing any substantial ballistic change.

While my invention is capable of being carried out in many different ways, for the purpose of illustration I shall describe only 45 one form of my invention hereinafter.

A powder made in accordance with my invention may be prepared in the following manner:—

A quantity of granulated nitrocellulose 50 powder is introduced into a revolving barrel provided with means for heating the same. A mixture of a nitro-hydrocarbon such as dinitrotoluene with camphor or with camphor and diphenylamin is introduced

into the barrel with the powder grains. The 55 barrel is then warmed sufficiently to partially liquefy the mixture of dinitrotoluene, camphor and diphenylamin, and held at this temperature for about 30 minutes, while the barrel is rotated to insure a uniform coating of the nitrocellulose powder grains with the mixture of dinitrotoluene, camphor and diphenylamin. The temperature of the barrel is then gradually raised to about 65° centigrade, and this temperature is maintained while the barrel is rotated from one to one and one-half hours to impregnate the nitrocellulose powder grains with the dinitrotoluene. During this latter rotation the excess camphor is driven off. The powder 70 grains if allowed to cool in this condition would adhere to one another so that a small amount of graphite is added, and the mixing continued until the powder has become dry, which takes about 20 minutes. An additional amount of graphite is then added and the glazing is continued until the powder grains no longer adhere to one another. The powder grains are then heated at about 45° centigrade for several days 80 until the odor of camphor disappears.

The dinitrotoluene used may be any one of the several isomers or it may be a mixture of isomers formed by the direct nitration of toluene. Pure dinitrotoluene which 85 is usually described as 1, 2, 4 isomer (o. p. dinitrotoluene) gives very satisfactory results. To lower the melting point of pure dinitrotoluene and also assist in bringing the dinitrotoluene into a high state of fluidity, 90 to promote the impregnation of the nitrocellulose powder grains with the dinitrotoluene, the dinitrotoluene is treated with a mixture of camphor and diphenylamin. Any suitable proportions of the impregnating 95 substances may be used, but I have found for example that a mixture containing 84 parts dinitrotoluene, 16 parts camphor and 4 parts diphenylamin provides an excellent impregnating composition. If 100 the nitrocellulose powder grains to be treated have been provided with incorporated diphenylamin as a stabilizer, the amount of diphenylamin used in the mixture may be decreased. The impregnating mixture having the diphenylamin therein has a still further advantage that any slight decomposition of the powder grains during

the impregnating operation, or later, is taken care of by the stabilizing action of the diphenylamin. The relatively high melting point of the dinitrotoluene is decreased by 5 the addition of camphor and diphenylamin to such a degree that it is possible to impregnate the powder grains at a temperature which is safe and convenient, and which will not effect the stability of the powder. 10 The impregnating mixture in the proportions above described becomes partially liquefied when it is warmed, and will be in a highly fluid state when the mixture is heated to a temperature of 65° centigrade, 15 whereas 1, 2, 4 dinitrotoluene melts at about 70.5° centigrade. The powder grains thus obtained will be found to be impregnated on their outer surfaces with dinitrotoluene, and their surfaces composed of nitrocellulose 20 colloided with dinitrotoluene, nitrocellulose colloided with camphor and dinitrotoluene, nitrocellulose colloided with dinitrotoluene, camphor and diphenylamin, or a mixture of any or all of these. The powder thus produced 25 produces a lower pressure initially at the breech of a gun and without producing an unduly high pressure along the barrel or at the muzzle. At the same time, it will also be found that the presence of the 30 material applied to the surface of the grains produces substantially no change in the velocity of the projectile. The fact that the coating material used penetrates the surface of the grains is very important as it is 35 found that many coating materials which do not penetrate the surface of the powder grains are liable to produce delay in ignition and are apt, furthermore, to produce powders too low in gravimetric density. By 40 the use of my invention the coated material is made to penetrate the powder grains sufficiently to form a dense surface which contains, however, sufficient nitrocellulose to be easy of ignition. Furthermore, the 45 powder so produced has practically no odor and is so slightly volatile that storage at the temperatures at which powders are stored produces substantially no ballistic change.

While I have described my invention 50 above in detail, I wish it to be understood that many changes may be made therein

without departing from the spirit of my invention.

I claim:—

1. A nitrocellulose powder grain having a 55 surface layer comprising a dinitrotoluene and camphor.

2. A nitrocellulose powder grain having a surface layer comprising a dinitrotoluene, camphor and diphenylamin. 60

3. A nitrocellulose powder grain having an impregnated surface comprising a solidified colloid containing a nitrotoluene, diphenylamin and nitrocellulose dissolved in a nitrotoluene. 65

4. A nitrocellulose powder grain having an impregnated surface comprising a solidified colloid containing a dinitrotoluene, diphenylamin and nitrocellulose dissolved in a dinitrotoluene. 70

5. A nitrocellulose powder grain having a surface comprising a solidified colloid containing a dinitrotoluene, camphor, diphenylamin and dinitrocellulose dissolved in a dinitrotoluene. 75

6. A nitrocellulose powder grain having a surface comprising a solidified colloid, containing nitrocellulose dissolved in a nitrohydrocarbon and camphor.

7. A nitrocellulose powder grain having a 80 surface comprising a solidified colloid containing nitrocellulose dissolved in a nitrohydrocarbon, camphor and diphenylamin.

8. A nitrocellulose powder grain having a surface comprising diphenylamin and a so- 85 lidified colloid containing nitrocellulose dissolved in a dinitrotoluene and camphor.

9. A nitrocellulose powder grain having a surface layer comprising dinitrotoluene and diphenylamin, with nitrocellulose dissolved 90 therein.

10. A nitrocellulose powder grain having a surface comprising dinitrotoluene, diphenylamin and camphor, with nitrocellulose dissolved therein. 95

In testimony that I claim the foregoing I have hereunto set my hand.

ARTHUR SAMUEL O'NEIL.

Witnesses:

EDWIN F. STIMPSON,  
VICTOR E. COMEGYS.